

[54] METHOD OF MAKING A SOLID-STATE SUPERCONDUCTING ELECTROMAGNETIC RADIATION DETECTOR

[75] Inventors: Myron Strongin, Center Moriches; Anand M. Saxena, Upton; Jack E. Crow, Bellport, all of N.Y.

[73] Assignee: The United States of America as represented by the United States Atomic Energy Commission, Washington, D.C.

[22] Filed: Apr. 4, 1973

[21] Appl. No.: 347,756

[52] U.S. Cl..... 324/43 R, 29/599, 307/306

[51] Int. Cl..... G01r 33/02

[58] Field of Search ..... 324/43 R; 29/599; 307/306

[56] References Cited

UNITED STATES PATENTS

3,290,186 12/1966 Rosi et al..... 29/599

3,325,888 6/1967 Weinig et al..... 29/599

FOREIGN PATENTS OR APPLICATIONS

1,196,788 7/1970 Great Britain..... 307/306

Primary Examiner—Robert J. Corcoran

Attorney, Agent, or Firm—John A. Horan; Leonard Belkin; Cornell D. Cornish

[57] ABSTRACT

Method for making a solid-state superconducting electromagnetic radiation detector by the steps of dividing aluminum into tangled, irregular, clusters of small randomly arranged oxide coated aluminum particles that are compressed and shaped into a self-sustaining solid mass. Connecting leads to the mass and cooling the mass to superconducting temperatures provides a transducer-detector that produces an output voltage in response to electromagnetic radiation that is incident on the surface of the mass over a broad band of frequencies.

8 Claims, 9 Drawing Figures



PATENTED JUL 16 1974

3,824,457

SHEET 1 OF 3



Fig. 1



Fig. 1a

PATENTED JUL 16 1974

3,824,457

SHEET 2 OF 3



Fig. 2



Fig. 3



Fig. 3a



Fig. 3b



Fig. 4



Fig. 5



Fig. 6

# METHOD OF MAKING A SOLID-STATE SUPERCONDUCTING ELECTROMAGNETIC RADIATION DETECTOR

## BACKGROUND OF THE INVENTION

This invention was made in the course of, or under a contract with the United States Atomic Energy Commission.

In the field of physics it is advantageous to detect low energy electromagnetic radiation over a broad band of frequencies from about 200 KHz upwardly. Various means and methods have been proposed or used for the desired detection, such as the detector used for radio astronomy at various laboratories and universities throughout the United States, but the receivers used heretofore have been large and cumbersome or they have been difficult or expensive to build or aim. It is additionally advantageous to provide compact microwave detectors and a method of making the same in a variety of shapes and sizes for the sensitive detection of microwaves over a broad band of frequencies.

It is an object of this invention, therefore to provide compact easy to build and operate radiation detectors and a method of making the same in a variety of shapes and sizes for the sensitive detection of radiation over a broad band of frequencies from about 200 KHz upwardly.

## SUMMARY OF THE INVENTION

This invention provides an easy to build and operate radiation detector and a method of making the same in a variety of shapes and sizes for detection over a broad band of frequencies above 200 KHz wherein the detector has a major amount of superconductor particles in a minor amount of an insulating sea. More particularly, this invention provides a method of dividing a superconductor into irregularly shaped randomly arranged superconductor particles having a thin insulating coating, and compressing the same into the desired shape and size for the sensitive detection of electromagnetic radiation at operating temperatures over a broad band of frequencies above 200 KHz. To this end, in one aspect the compressed mass forms a plurality of continuous intertwined, non-uniform cross-section, superconductor filaments having a critical current density of the order of  $10^{-5}$  to  $10^{-6}$  amps per sq. centimeter, wherein small cross-section weak mechanical-electrical links having a diameter of below about 100 Å connect to larger cross-section strong mechanical-electrical links having diameters of  $\sim 100$  - 600 Å that are arranged in continuous intertwined chains of alternate periodic weak and strong links having a mass resistance of at least  $3 \times 10^3$  ohm-cm.

In one embodiment, the method of this invention comprises dividing an aluminum ingot into cubes by cutting, cleaning the cubes by etching, evaporating the cleaned cubes in a chamber containing a protective atmosphere, depositing the evaporated material on the inside surface of a sphere inside the chamber by condensation to form irregular-shaped, randomly arranged particles having an average cross-sectional width of between about 100 to 600 Angstroms (Å), coating the particles completely and uniformly with an aluminum oxide layer on a major amount of the aluminum by exposing the particles to an oxygen containing gas, collecting the coated particles into tangled, irregularly

shaped, randomly arranged clusters, compressing the tangled clusters to interlock them together in a solid shaped mass, finishing the mass by connecting leads thereto, and cooling the finished solid to operating temperatures. With the proper selection of steps and conditions, as described in more detail hereinafter, the desired detector and detection is achieved.

The above and further novel features and objects of this invention will be apparent from the following detailed description of one embodiment when read in connection with the accompanying drawings, and the novel features will be pointed out in the appended claims.

## BRIEF DESCRIPTION IN THE FIGURES

FIG. 1 is a partial cross-section of the apparatus of this invention for performing the method thereof; FIG. 1a shows the detector;

FIG. 2 is a graphic representation of the number of particles vs particle diameter of this invention that were employed in one example of the detector of this invention;

FIG. 3 is a partial three-dimensional view of one embodiment of a detector made by the method of this invention and the apparatus of FIG. 1; FIG. 3a is a partial three-dimensional view of the filaments of this invention; and 3b is a partial three-dimensional view of the intertwined, interlocked chains and filaments of this invention, having proximate boundaries therebetween.

FIG. 4 is a partial detailed view of the particles and clusters of the detector of FIG. 3;

FIG. 5 is a graphic representation of the voltage output vs temperature of the detector of FIG. 3 after the particles of FIG. 4 had been compacted, assembled and cooled to operating temperatures in accordance with this invention;

FIG. 6 is a graphic illustration of the resistance of the detector of FIG. 3 vs temperature.

## DETAILED DESCRIPTION OF ONE EMBODIMENT

This invention is useful in making inexpensive, compact, easy to fabricate and operate radition detectors in a variety of shapes and sizes for the sensitive detection of electromagnetic radiation over a broad range of frequencies. These frequencies, for example, are above 200 KHz. As such this invention is useful in the field of radioastronomy, but it is also has a wide utility in any application where such detection is required, since this invention provides a detector that is sensitive to weak radio or other low power level electromagnetic radiation. Thus, this invention is useful in the field of physics generally, as well as in the field of radioastronomy particularly, as understood hereinafter from the detector 9 of FIG. 1a.

Referring to FIG. 1, a glass bell jar 10 is sealed from the ambient atmosphere and evacuated through a suitable exhaust 12 having a conventional vacuum pump (not shown) after a sample of an aluminum cube 14 is placed in filament 26 inside glass sphere 16, which is located inside the bell jar 10. After evacuation, the bell jar 10 is pressurized to a pressure indicated by gauge 18 from a conventional protective He source through pipe 22 and valve 24. A current source connected to filament 26 through leads 28 then boils off the aluminum from the sample 14, which was placed inside of the filament. FIG. 2 shows the particle sizes produced.

The aluminum cube is evaporated from the filament 26 and deposited in irregularly shaped, randomly arranged, aluminum particles on the inside of the glass sphere 16, and the described aluminum particles are removed from the glass sphere and formed into tangled, irregularly shaped, randomly arranged clusters. The particles are then coated completely and uniformly with  $\text{Al}_2\text{O}_3$  by exposure to  $\text{O}_2$ . To this end, the particles are brushed from glass sphere 16 into a suitable container in an oxygen containing ambient that forms the  $\text{Al}_2\text{O}_3$  coating on the particles. The ambient air is used for this. The number of particles vs average particle size recovered is illustrated by FIG. 2. Herein, the sizes used are the maximum cross-sectional dimension.

As seen in FIG. 3, the coated particles 32 are collected randomly in a mold 33 cylindrically shaped and compressed at 1,000-5,000 psi, where, as illustrated in FIG's. 3a, 3b and 4, there are formed a solid mass 34 consisting of interlocked chains 47 of non-uniform cross-section aluminum filaments 41, having boundaries 51 therebetween, as described in more detail hereinafter. The relative size of the interlocked particle clusters 36 and the interlocked particles 32 are illustrated in FIG. 4. Suitable leads 37 applied to the opposite ends of the solid mass 34 provide the finished detector 9, which is operable when cooled in a cryostat 39, as shown in FIG. 1a. Means 40 send the radiation, and volt meter  $v$  shows the voltage.

It will be understood from the above that the process of this invention compresses the particles and clusters into a plurality of continuously interlocked and intertwined, non-uniform cross-section, aluminum filaments 41. These filaments have a critical superconducting transition current density of about  $10^{-5}$  to  $10^{-6}$  amps per square centimeter. As shown in FIG. 3a the filaments 41 have weak mechanical and electrical links 43 forming aluminum filaments below about 100 Å in cross-section connecting larger cross-section aluminum filaments between about 100 - 600 Å arranged as strong links 45 in continuous intertwined chains 47 of alternate periodic strong and weak links. For purposes of this application, weak links are aluminum filaments having a cross-sectional diameter of below about 100 Å, and strong links are like aluminum filaments having a cross-sectional diameter of about 100 - 600 Å.

In operation, the voltage output of the solid mass 34 vs temperature is illustrated in FIG. 5. The solid mass 34 is cooled to within 1° of the  $\text{Al}$   $T_c$ , and the leads 37 are connected to conventional circuitry, such as a voltmeter, for determining the voltage output from the detector 9 in response to incident electromagnetic radiation on the surface of the solid mass 34. FIG. 6 illustrates the resistance vs temperature of the detector of FIG. 3.

Examples of the method and apparatus employed in making one embodiment of the detector 38 of FIG. 3 are as follows:

#### EXAMPLE I

A standard water-cooled carborundum saw divided an aluminum ingot into small cubes about 2 - 3 millimeters on a side. Etching in 70 pts  $\text{H}_3\text{PO}_4$ , 12 pts  $\text{CH}_3\text{COOH}$ , 3 pts  $\text{HNO}_3$ , and 15 pts  $\text{H}_2\text{O}$  then removed any surface contamination from the aluminum (purity 99.9 Percent).

The aluminum was placed in a helical tungsten filament inside a vacuum chamber which was evacuated to

$1-5 \times 10^{-6}$  mm of Hg. The system was then filled to a pressure between 1-5 mm of Hg with helium or other inert or protective atmosphere. The aluminum division proceeded further by evaporating the etched cube from the helical tungsten filament. The aluminum was deposited on the inside of the glass sphere to form irregular, randomly arranged particles averaging about 100 - 600 Å in diameter. The evaporation rate was controlled manually utilizing a variac that fed a standard low voltage, high current transformer connected to the filament. The evaporation and depositing was continued until all the aluminum in the etched cube has boiled off, and then the system was allowed to cool to room temperature before the vacuum (vacuum bell jar) was vented to the atmosphere.

The venting to the oxygen containing ambient coated the deposited particles with a thin minority layer coating of an insulating oxide with a major portion of the aluminum remaining. These coated particles were collected into tangled, irregular, randomly arranged clusters by brushing or scraping them into a collecting container. The particles were then transferred to a mold where shaping and linking of the clusters was achieved by compression of about 1,000 psi into the desired shaped solid mass containing the plurality of intertwined, non-uniform cross-section, superconductor filaments having a critical superconducting transition current density of about  $10^{-5}$  to  $10^{-6}$  amps per square centimeter, wherein weak links below about 100 Å connected strong links between about 100 - 600 Å arranged in continuous intertwined and interlocked chains of alternate periodic strong and weak links, as determined visually.

Electrical leads were attached either by silver painting or pressing to finish the detector. Upon cooling the finished detector in a cryostat to an operating temperature at least as low as 1.3 - 1.4 K (the critical superconducting temperature  $T_c$  of aluminum being 1.19 K) and exposing the surface of the shaped, solid, cooled mass to electromagnetic radiation of 200 KHz or higher, a D.C. voltage was detected across the leads. Actual voltages were detected between 200 KHz and 4 GHz below 1.3 - 1.4 K. The radiation was applied in this example by a coil around the solid mass of cylindrical sample with the ends of the coil connected to a continuously variable frequency and amplitude rf oscillator.

#### EXAMPLE II

The steps and conditions of Example I were repeated using various gas pressures using both helium and residual gases such as oxygen and water vapor during the evaporation step to determine the effect on the particle and cluster size. It was found that the particle and cluster size up to an order of magnitude larger than the mean particle size could be controlled by varying the protective gas pressure during the evaporation.

#### Example III

The steps and conditions of Example I were repeated using various gases such as Ar, Xe, Kr and lighter gases during the evaporation step to study the effect of different molecular weight or size of the gas molecules on particle size. For comparable conditions, He gas gave the smallest particles and best results, and was determined to be the best gas, although Ar, Xe or Kr could also be used alone or in combination.

## Example IV

The steps and conditions of Example I were repeated at various substrate and collection surface temperatures and it was found that satisfactory results, comprising the desired particles, particle sizes, and clusters were obtained at incrementally increasing filament temperatures starting at the melting temperature of aluminum with the collection surface temperature approximately equal to room temperature of about 72° F. The currents used to melt the aluminum cube were typically about 100 Amps a.c. Upon melting at 100 Amps, the aluminum was retained along the filament by surface tension. The current was then further increased about 1 amp every 1-2 minutes to achieve the evaporation. This evaporation took about 2-5 minutes for an aluminum cube having a mass of 2 - 3 grams.

## Example V

The steps and conditions of Example I were repeated at slow evaporation rates. It was determined that after the aluminum melting point was reached, that by not increasing the current further the result was that there was too low of an evaporation rate to form aluminum particles, because of the presence of small reactive gases in the bell jar. For example, an evaporation rate of more than  $\frac{1}{2}$  hour had the effect of not producing particles, i.e., the aluminum coated the inside of the glass sphere on which it was condensed.

## Example VI

The steps and conditions of Example I were repeated for various compaction pressures to produce inhomogeneously interlocked and compacted clusters and particles. It was found that the resistance of the aluminum superconductor decreased at about 1.3 K as the compaction pressures increased from 500 to 5000 psi. In this example, at 1.3 K the resistivity of the compacted sample was  $10^6$  ohm-cm,  $3 \times 10^3$  ohm-cm, 100 ohm-cm at compaction pressures of 400 psi, 1,000 psi and 5,000 psi. At the superconducting critical transition temperature  $T_c$  of the sample, the optimum resistivity was  $\sim 103 - 300$  ohms-cm.

## Example VII

The steps and condition of Example I were repeated to show the effect of decreasing the temperature of the cryostatically cooled cylindrical detector. It was found that for a given radiation input incident on the outside cylindrical surface of the detector that an increasing positive voltage output was produced, which increased as the temperature decreased from about 1.35 K to about 1.0 K as shown in FIG. 5; also, the voltage output level was substantially constant from 25 MHz to at least 400 MHz. A slightly increasing voltage output was produced by incident radiation from 200 KHz to as high as 8 GHz.

## Example VIII

The steps and conditions of Example I were repeated in various molds without decreasing the sensitivity of the detector produced. Cylindrical detectors of various sizes were made, but many other rounded or flat shapes, such as spherical, square, disc, or rectangular, could be satisfactorily made and used.

It was found that, by compacting  $\approx 300$  A A1 particles in the form of clusters the composite material was

composed of greater than  $10^{12}$  junctions that behaved coherently when exposed to rf surface radiation. In these large arrays with a large number of junctions, a steady state dc voltage of up to 200  $\mu$ V was observed from the leads connected to the compressed solid mass or particles even with zero dc bias voltage applied to the detector. This was in contrast to the behavior of a single junction with a zero bias voltage present, where it was found that the single junctions switched between different quantum stages. FIG. 6 shows the resistive transition of the array of particles in the detector. The transition has a long tail, this behavior is ordinarily characteristic of weakly linked cooperative systems, which are extremely current sensitive

It was also found that the dc output voltage from the detector varied as a function of frequency for constant amplitude rf incident energy. By effectively changing the coupling of the radiation to the detector with a tuning stub, which was similar in function to the ones shown in FIG's 13-16 U. S. Pat. No. 3,530,332, by Giordano, or by changing the frequency tuning, the voltage sign could be made to change from plus to minus.

The radiation power input in this example followed that of the others, where this input was less than a microwatt. In the cylindrical detector of this example, where the cylinder was 1/4 inch in diameter, the response was good for a number of tests from 1 MHz to 4 GHz, although higher frequencies or lower frequencies down to about 200 KHz were also possible. The upper limit has not been established yet. In general the resistance of a 1 inch long longitudinally extending cylindrical detector made in accordance with this example (about 1 inch long and about 1/4 inch in diameter) was about 1,000 ohms at 4.2 K, which was well above the critical superconducting temperature of the aluminum in the detector. To make the measurements, a sample detector was mounted below a shorted section of  $50 \Omega$  rf cable, or in a waveguide terminated by a  $50 \Omega$  termination.

## Example IX

A detector was fabricated in the same way as described in Example I, except that after the particles were removed from the bell jar and before they were compressed, any existing particle clusters were broken up. The breaking up of the particle clusters was achieved by passing a colloidal solution of the particles suspended in methanol through a closely fitted piston and cylinder. The piston was rotated at a high velocity and the cylinder remained stationary as the colloid was forced between the piston and cylinder; the resulting shear waves produced in the liquid broke the particle clusters. The separated particles were collected by allowing the methanol to evaporate leaving the particles as a residue. The individual particles were then treated similarly to Example I with the additional exception that a larger pressure was required in the molding process to attain the desired resistivity of the detector. This process had the advantage that the higher pressure used in the molding process resulted in a sample which was less susceptible to damage during handling.

In the above examples it was not completely understood by the large cross-section, inhomogeneous interlocking of irregularly shaped particles and clusters under compression produced the desired results without biasing, nor why the weak small cross-section, fila-

mentary, superconductor links between the particles didn't cancel but acted synchronously and coherently with enhanced sensitivity as they did, but it is theorized that the inhomogenous junction array internally was shaped to form a coherent cooperative system of Josephson and/or other junctions independently of the specific solid mass shape selected, wherein the sign of the voltage was determined by an initial asymmetry. In contrast, individual junctions are similar to a single magnetic dipole, which has no preferred magnetism or which alone can flip between spin stages. However, when magnetic dipoles are together, the system makes a transition to coherent state so as to produce a steady stage magnetic polarization commonly referred to as a ferro-magnetic state.

Many arrays of weak links were believed to have been made by the described process with individual particle clusters where the individual particles were about 300 Å across to provide  $10^{12}$  or more junctions on the macroscopic scale. Besides the enormous structure in the  $dT/dV$  vs  $V$  characteristic, a striking property of the superconducting state was that when rf radiation impinged on unbiased samples, a constant dc voltage of up to 200  $\mu$ V or more appeared that was stable in time and dependent on the frequency range of at least from 1 MHz to 4 GHz, in contrast to the switching of single junctions in sign and voltage output magnitude.

Looking at the detector as an alloy, the superconducting aluminum provided a majority aluminum constituent in sea of aluminum oxide forming a normal resistance insulator matrix of aluminum oxide forming a minority constituent and proximate boundaries  $<500$  Å across the boundaries. Thus, as shown in FIG. 3b, a plurality of interstitial boundaries 51 could exist between the continuous, intertwined chains of non-uniform cross-section, superconductor filaments 41, and these boundaries could in some cases individually conduct by tunneling.

While the above has described the use of aluminum particles having an oxide coating thereon for forming the detector of this invention, it will be understood that other superconducting metals having oxide coating thereon can be used. For example, tin particles having a tin oxide coating thereon can alternately be used. In this case the operating temperature would be higher than with the Al particles due to the fact that the superconducting transition temperature of the array would be near 3.7° K. Other examples, would employ oxide coated niobium particles, where the superconducting transition temperature, i.e., the  $T_c$ , is near 9° K.

This invention has the advantage of providing a detector and method for making it for detecting radiation from 200 KHz upwardly over a broad band of frequencies up to at least 8 GHz at a wide variety of amplitudes as weak as those contemplated for radioastronomy purposes. Moreover, the detector of this invention is small, compact, easy to assemble and operate, and has any ordinary shape that is desired, such as cylindrical, rounded, rectangular, disc-shaped, etc.

What is claimed is:

1. Method for making a solid, solid-state, electrically non-biased, mechanically self-sustaining non-adjustably clamped, superconducting electromagnetic

radiation detector that is substantially without interstitial spaces while being sensitive at between 1.3 to 1.4 K to the presence of an electromagnetic radiation input of at least 200 kHz, comprising the steps of:

- 5 a. collecting irregularly shaped, randomly arranged resistive particles of average cross-section in the range of 100 – 600 Å of aluminum having a purity of 99 percent coated with  $Al_2O_3$  into tangled, irregular, randomly arranged resistance clusters;
- b. compressing the resistive clusters at sufficient pressure resistively to interlock the particles so as to produce resistive mechanical and electrical links between adjacent particles having a resistance of  $3 \times 10^3$  ohm-cm and a critical superconducting transition current density of between about  $10^{-5}$  to  $10^{-6}$  amps/cm<sup>2</sup>, said links averaging predominantly 100 Å or below in cross-section said compressed particles forming a solid mechanically self sustaining mass upon removal of the pressure;
- c. connecting electrical output leads to separated portions of the compressed clusters; and
- d. cooling the compressed clusters to a temperature of within 1°K of the critical superconducting transition temperature  $T_c$  of said aluminum.
2. The method of claim 1 in which said clusters are compressed at a pressure in the range of from 1,000 to 5,000 psi.
3. The method of claim 1, in which the collecting is by the evaporating of said aluminum from a heated tungsten filament followed by the condensation of the evaporated aluminum on the inside surface of a container holding a helium atmosphere containing residual oxygen.
- 35 4. The method of claim 1, in which said step of compressing said tangled, irregular, randomly arranged clusters interlocks the same in a multiplicity of continuous interlocked chains of periodic alternate strong and weak links forming non-uniform cross-section superconductor filaments.
5. The method of claim 1, including the step of detecting a voltage output from said solid mass in response to an electromagnetic radiation field at the surface of the mass at a frequency of at least 200 KHz where the mass is cooled to an operating temperature within 1° K of the temperature where the resistance rapidly decreases to the superconducting transition temperature of the aluminum particles.
6. The method of claim 1 in which said compressing is in a mold under a compacting pressure of up to about 5,000 pounds per square inch that forms a cylindrical body in said mold.
7. The method of claim 3 in which said particles are evaporated and condensed on a surface at an average size of between about 100 to 600 Angstroms.
- 55 8. The method of claim 7 in which an  $Al_2O_3$  coating is formed on the aluminum particles by surrounding said particles with an oxygen containing ambient to produce a coating thereon, said coated particles being compressed so that upon said compression said coated particles provide a mass containing a major amount of a first aluminum superconductor component in a matrix of a minor amount of a second  $Al_2O_3$  normal resistance component.

\* \* \* \* \*